# EUROPEAN PATENT SPECIFICATION

(11) **EP 1 594 686 B1**
(45) Date of publication and mention of the grant of the patent: **26.03.2008**
(21) Application number: 03796989.6
(22) Date of filing: 12.12.2003
(51) Int. Cl.: B32B 3/02, B32B 33/00, D03D 27/00, D04H 11/00, D05C 17/00, D06B 11/00, D02G 3/40

(54) **ENHANCED SURFACE COVERINGS AND METHOD**
VERSTÄRKTE OBERFLÄCHENBESCHICHTUNGEN UND VERFAHREN
REVETEMENTS DE SOLS AMELIORES ET PROCEDE CORRESPONDANT

(30) Priority: 23.12.2002 US 327724; 05.09.2003 US 500529 P; 11.12.2003 US 732937
(43) Date of publication of application: 16.11.2005
(73) Proprietor: Milliken & Company, Spartanburg, SC 29303 (US)
(72) Inventor: BRIDGES, James, C., LaGrange, GA 30240 (US); LATHAM, Wilson, A., Alma, GA 31510 (US); LASSETER, David, M., Alma, GA 31510 (US); MCCARTY, David, E., Alma, GA 31510 (US); DEEN, Carroll, E., Nicholls, GA 31554 (US)
(74) Representative: HOFFMANN EITLE
(86) International application number: PCT/US2003/039626
(87) International publication number: WO 2004/061189

(56) References cited:
- EP-A- 0 359 881
- EP-A- 0 444 637
- WO-A-99/14408
- WO-A1-88/03969
- US-A- 5 035 018
- US-A- 5 116 243
- US-A- 5 567 256
- US-A- 5 903 962
- US-A1- 2002 034 607
- US-A1- 2003 014 823

## Description

### BACKGROUND OF THE INVENTION

The present invention relates to a process for manufacturing an improved or enhanced surface covering such as a carpet and the carpet manufactured thereby. More specifically, the present invention relates to a process for forming a carpet wherein the carpet comprises a combination of fibers with at least one fiber being lower melting than the other fiber or fibers and printing or dyeing this carpet. The invention also relates to a carpet and related formation process wherein the carpet includes pile yarns including a combination of wool fiber and at least one low melt polymeric fiber constituent having a melting point such that it may be heat activated to at least partially fuse the wool fibers together thereby enhancing printability and reducing shedding of the wool during use.

It has been known in the art to combine various yarns to form a composite yarn for carpet production. Examples of such teachings include U.S. Pat. No. 5,336,562, issued to Forero, wherein polyethylene filaments and polypropylene filaments are combined in a "parallelized" orientation. The parallel fibers are then heated to an excess of 120°C to melt the polyethyelene filaments. Yarns such as these are dyed prior to incorporation into a carpet. Dyeing prior to carpet formation, weaving or tufting, is highly undesirable since inventory must be maintained for each fiber color. Furthermore, the ability to custom manufacture carpet and the selection of designs and patterns is severely hindered.

Other yarns have been used to manufacture carpet in either a colorless form or in a generic color. The carpet is then overcoated with a pattern, or color, by printing or dyeing, on demand. This process greatly decreases the items that must be maintained in inventory and thereby decreases manufacturing cost. A superior form of jet dyeing of carpet in a pixelated fashion has been achieved using a Millitron^{™} jet dye machine by Millken & Company of Spartanburg, South Carolina. Techniques for printing carpet are known and exemplified in U.S. Pat. Nos. 3,894,413; 5,142,481 and 6,120,560. While these methods have greatly increased the manufacturing efficiency, the pattern resolution is limited, in part, by carpet sueding. Carpet fibers have a tendency to bend or lay over. If the pile or yarns are not all oriented similarly, one section may appear to be a different shade than the surrounding area. While this is common in finished carpet the ability of a carpet to suede or for the pile to be oriented other than vertical greatly decreases the resolution of any image that can be printed or dyed on the carpet. If for example, two regions are sueded differently the dye will be partially applied to the side of the sueded fibers instead of at the tuft head, or top, of the fiber. Therefore, the limiting resolution of the printing process is determined, in part, by the ability of the carpet to suede, pile lay, pile orientation, etc.

Sueding can be eliminated, or mitigated, by increasing the brittleness of the carpet fibers. This is contrary to desires in the art since the more brittle carpet is considered to be deficient with respect to comfort factors typically desired in carpet. For example, a harder or more brittle carpet may not be viewed as soft or plush.

Yet another problem in the art is the inconsistency with which carpet fibers absorb dye. One approach to circumvent this deficiency is to utilize ever softer fibers which absorb dyes more readily. Softer fibers have a higher tendency to suede and therefore resolution is still limited.

Still another problem which has been encountered in carpet manufacturing has been in the shedding of carpet fibers when the pile yarn incorporates high percentages of wool. While wool is soft and provides a plush luxurious pile, it has been common that fibers within the pile yarns tend to shed away from the yarn during use. This results in the undesirable accumulation of large quantities of loose wool fiber across the surface of the carpet which must be frequently removed by vacuuming. Such shedding also results in the gradual degradation of the pile thereby reducing the overall pile density. Further examples of producing carpets are disclosed in WO-A- 99/14408 and US 2002/0034607.

There has been a long felt desire in the art for a carpet, and a process for preparing carpet, wherein the carpet can be printed or dyed to a high degree of definition, or high resolution, yet which still has the features associated with comfort.

### BRIEF SUMMARY OF THE INVENTION

According to the present invention there is provided a process for forming a jet dyed carpet comprising: forming at least one higher melting thread comprising at least one higher melting point fiber constituent, wherein the higher melting point constituent is non-continuous; passing said higher melting thread through a doubling or winding process wherein a lower melting point thread is added; spinning or twisting the higher melting thread and the lower melting thread to form a combined thread; heating said combined thread above a temperature sufficient to melt said low melt thread; tufting said thread in the carpet backing to form the tufted carpet; and printing an image on said tufted carpet with a jet dye machine.

According to the present invention there is provided a jet dyed carpet comprising: at least one higher melting thread comprising at least one higher melting point fiber constituent, wherein the higher melting point constituent is non-continuous and a lower melting point thread added through a doubling or winding process, wherein the higher melting thread and the lower melting thread are spun or twisted to form a combined thread, wherein the combined thread is heated above a temperature sufficient to melt said low melt thread, wherein the combined thread is tufted in a carpet backing to form a tufted carpet; and wherein an image is jet dyed on the tufted carpet with a jet dye machine.

It is an object of at least one embodiment of the present invention to provide a carpet, and process for manufacturing the carpet, which allows for high resolution printing or dyeing and that maintains high resolution after wear.

It is another object of at least one embodiment of the present invention to provide a carpet, and process for manufacturing the carpet, which has excellent wearability and a durable high resolution image.

It is another object of at least one embodiment of the present invention to provide a carpet, and process for manufacturing the carpet, which allows for the use .of high wool content pile yarn while reducing the occurrence of shedding.

A particular feature of at least one embodiment of the present invention is the ability to decrease inventory while still being able to provide carpet with a pattern that is selected on demand and wherein the pattern is a high resolution pattern that is durable and remains high resolution after wear.

These and other advantages are provided in selected process for forming a carpet, and the carpets formed thereby. A first process includes forming a thread or yarn comprising low melt fiber or filament and high melt fiber or filament. The thread is then heated (heat set) above as temperature sufficient to melt the low melt fiber. The thread is tufted in a carpet backing to form a tufted carpet. The tufted carpet is then printed or dyed with an image.

In accordance with another embodiment of a process for forming printed or dyed carpet, and the carpet formed thereby, the process comprises the steps of forming a blended fiber comprising at least one low melt fiber and at least one high melt fiber. A thread or yarn is formed of the blended fiber. The thread is heated above a temperature sufficient to melt the low melt fiber. The thread is tufted in a carpet backing to form a tufted carpet. Then, an image is printed or dyed on the tufted carpet.

In yet another embodiment of a process for forming printed carpet, and the carpet formed thereby, the process comprises the steps of forming a thread or yarn from at least one high melt fiber. The thread is passed through a doubling or winding process wherein at least one low melt fiber is incorporated into the thread. The combined thread is heated above a temperature sufficient to melt the low melt fiber. The heated thread is tufted in a carpet backing to form a tufted carpet. Then, an image is printed or dyed on the tufted carpet.

In still another embodiment of a process for forming printed carpet, and the carpet formed thereby, the process comprises the steps of forming a thread from a high melt fiber, passing the thread through a ring spinning process wherein a low melt fiber is incorporated into the thread. Next, the thread is heated above a temperature sufficient to melt the low melt fiber. The thread is tufted in a carpet backing to form a tufted carpet. Then, an image or pattern is printed on the tufted carpet.

Still another process includes forming a yarn comprising wool in combination with a low melt fiber or filament constituent. The yarn is then heated (heat set) above a temperature sufficient to melt the low melt fiber such that the low melt fiber provides a degree of fusion bonding between at least a portion of the wool fibers. The yarn is tufted in a carpet backing to form a tufted carpet. The tufted carpet is then dyed or printed with an image.

In another embodiment the process comprises the steps of forming a thread or yarn from wool fibers. The thread is passed through a doubling or winding process wherein at least one low melt fiber is incorporated into the thread or yarn to form a heat fuseable yarn structire. The heat fuseable yarn structure is heated above a temperature sufficient to melt the low melt fiber and fuse at least a portion of the wool fibers together. The fused yarn structure is tufted in a carpet backing to form a tufted carpet. Then, the tufted carpet is dyed or printed.

In still yet another embodiment the process comprises the steps of forming a thread or yarn from wool fiber, passing the thread through a ring spinning process wherein a low melt fiber is incorporated into the thread or yarn to form a heat fuseable yarn structure. Next, the heat fuseable yarn structure is heated above a temperature sufficient to melt the low melt fiber and fuse at lest a portion of the wool fibers together. The fused yarn structure is is tufted in a carpet backing to form a tufted carpet. Then, the tufted carpet is dyed or printed.

In accordance with at least one embodiment of the present invention, the addition of a "low melt" polyester or nylon fiber or filament (such as manufactured by Solutia) during the yarn manufacturing process results in a yarn after the heatset process that has enhanced fiber cohesion as well as improved end point definition and optical color evenness when put into a carpet base and dyed by a jet dye machine. Both stape and filament low-melts will work but the filament low-melt is preferred.

It is contemplated that even after extended wear tests, the carpet of the present invention shows less evidence of "sueding" - a phenomenon in typical carpet where over time the yarn bundles begin to weaken and bend, resulting in wear on the non-tip surface of the yarn resulting in worn/pulled/broken fibers. These broken fibers give a muted appearance to the carpet which changes to another shade when a hand or vacuum is run over the carpet (hence the term "sueding"). Embodiments of the present invention reduces this problem.

In addition, it is contemplated that the carpet of the present invention may be characterized by reduced fiber shedding of the wool fiber consituent due to the fusion bonding by the low melt constituent. A reduction in fiber shedding, in turn, reduces fiber loss over time and increases overall life.

Additionally, the yarn of the present invention may enhance any jet dyeing operation due to the nature of the yarn being more erect in the carpet at the dyeing process, hence the dye which is streamed to exact points on the carpet face is more apt to be applied where, and in the quantities, intended.

Embodiments of the invention enhance the dyeability of carpet, the appearance of the carpet over time, both the color and the patterning detail, and the life of the yarn bundle itself.

In at least one embodiment, the present invention provides one or more of the following advantages:

1) Extends the effective life of carpet, an advantage for the consumer and an environmental enhancement (less landfill, less recycling.)

2) By being added at the beginning of the product cycle, eliminates the need for elaborate rollers, steaming and the like at pre-dyeing to stand the fiber-bundles upright for dyeing.

3) Enables greater detail in dyeing patterns when combined with proprietary dyeing processes such as the Millitron^{™} jet dye machine.

4) Addresses the "sueding" problem eliminating the need for post installation shearing of carpet to remove broken or loose fibers to return the original appearance to the carpet.

5) Addresses shedding thereby reducing the rate of wear and the frequency of required vacuuming.

In accordance with at least one embodiment, the present invention allows for the twist lock of multiple yarn plies together, reduces sueding of spun carpets, and allows an insert fiber to be added to yarn on existing equipment and processes.

### BRIEF DESCRIPTION OF THE DRAWINGS

For a better understanding of the present invention and to show how the same may be carried into effect, reference will now be made, by way of example to the accompanying drawings, in which:

Fig.1A is a block diagram illustrating, schematically, an exemplary carpet manufacturing process of the present invention.

Fig. 1B is a block diagram illustrating, schematically, a second exemplary carpet manufacturing process of the present invention.

Fig. 2A is a schematic representation of a thread comprising fibers prior to heat set.

Fig. 2B is a schematic representation of a thread comprising fibers after heat set.

Figs. 3A-B are schematic cross-sectional representations of tufted carpet wherein the fibers are intermingled in Fig. 3A and discrete in Fig. 3B.

Figs. 3C-D are respective, schematic, top view representations of the tufted carpet of Figs. 3A-B wherein the tuft heads, are intermingled in Fig. 3C and discrete in Fig. 3D.

Fig. 4 is a block diagram of a first preferred process for preparing fibers of the present invention.

Fig. 5 is a block diagram of another preferred process for preparing fibers of the present invention.

Fig. 6 is a block diagram of yet another preferred process for preparing fibers of the present invention.

Fig. 7 is a block diagram of a substrate pattern dying process and apparatus embodying at least one embodiment of the instant invention.

Fig. 8 is a cross-sectional schematic depiction of a solid shade dyer of a kind that may be used to practice the instant invention.

Fig. 9 is a schematic diagram of a textile patterning device that uses a plurality of computer controlled discrete streams of liquid dye arranged in a series of color-specific arrays that span the path of the moving substrate to be patterned; and, it represents one Example of a patterning means useful in the practice of the instant invention.

### DETAILED DESCRIPTION OF THE INVENTION

In accordance with at least one embodiment of the present invention, a process for manufacturing a carpet that greatly increases manufacturing efficiency and the resolution with which a durable image can be printed or dyed on the carpet has been discovered.

In accordance with at least one preferred embodiment, the present invention is directed to a carpet comprising a composite fiber, thread or yarn printed or dyed in pixelated form. The composite fiber, thread or yarn comprises a low melt fiber and at least one high melt fiber.

Exemplary processes for manufacturing a tufted carpet will be described with reference to Figs. 1A and 1B. With reference to Fig. 1A, the primary carpet fiber such as nylon, wool or wool blend is initially prepared for use, at 200, as known in the art. The primary carpet fiber is preferably a standard or high melt nylon, wool or a blend of high melt nylon with wool. Although nylon (polyamide, nylon 6 or nylon 6,6), wool, or nylon wool blends are preferred, it is contemplated that any natural or synthetic fiber or filament or blend may be used. By way of example only, one contemplated blend which incorporates a relatively high wool content contains about 25% high melt point nylon blended with about 75% wool. Another contemplated primary carpet fiber blend contains about 80% nylon and about 20% wool. Of course, blends with higher and lower percentages of high melting point nylon and wool ranging from 100% high melting point nylon to 100% wool may likewise be utilized in the primary fiber. The primary fiber is blended with adjuvants or additives as desired, at 201. In one embodiment, illustrated in Fig. 1A, a low melt fiber 202 is incorporated with the primary fiber as a blend at 201. The blended fiber is then manufactured into a thread or yam, at 203. Alternatively, in a preferred embodiment, a low melt fiber 204 is incorporated with the thread or yarn during the yarn manufacture as indicated at 203 of Fig. 1B.

With reference to Figs. 1A and 1B, the resultant yam, comprising a high melt polymeric fiber constituent and/or wool fiber constituent and at least one secondary low melt fiber constituent, is heat set. The heat set temperature is chosen to be sufficiently high to melt the low melt fiber but not high enough to damage the wool or melt any high melt polymeric fiber. For the purposes of the present invention, the preferred low melt fiber has a melting point below about 160°C and the preferred high melt fiber has a melting point above about 160°C.

Next, the heat set yarn or thread is tufted into a carpet backing as illustrated at 206. The tufted carpet is then printed or dyed, preferably by a pixelated printing system which will be more thoroughly described herein.

The heat setting or heat fusing of the yarn comprising at least one high or standard melt fiber and at least one low melt fiber is theorized to create tie points between fibers or filaments. The result is a thread or yarn which has less spread, particularly at the end or yarn head, and which can, for example, be used in a higher density in the carpet. A schematic representation of the threads prior to heat set is provided in Fig. 2A and after heat set in Fig. 2B. It is observed that the high melt and low melt fibers, 301 and 302, are independent intermingled fibers prior to heat set but tied together, presumably at tie points, 303, after heat set. The low melt fiber is theorized to at least partially melt and adhere to the high melt fiber or fibers. Upon cooling the adhesive bonds remain.

The advantages of heat setting a thread comprising one or more low melt fibers and one or more high melt fibers and/or wool is illustrated schematically in Figs. 3A-D. Fig. 3A is a side view representing a cross-sectional cut of a tufted carpet tufted with a conventional yarn without low melt fiber, while Fig. 3B is a similar view representing the tufted carpet of the present invention with yarn with low melt fiber. Fig. 3C is a top view of the yarn of Fig. 3A and Fig. 3D is a top view of the yarn of Fig. 3B. As can be seen, the upper surface of the yam, or yarn head, is more compact when low melt fiber is incorporated with the wool, wool blend or high melt fiber followed by heat set. In other words, the yarn bundle is more cohesive, tighter, and more erect. The more compact area allows a finer tufting and print pattern. A diffuse upper surface, as illustrated in Fig. 3C, comprises fibers from adjacent threads or yarns which are intermingled. When a high resolution pattern is printed or dyed thereon, the individual fibers from adjacent yarn will be translationally mobile thereby diffusing the high resolution image. For this reason, the resolution with which carpets could be printed or dyed has been previously limited.

Also, after wear, the conventional tufted carpet of Figs. 3A and 3C would even be more fuzzed, dispersed, frayed, will have even less resolution, and the like. In contrast, the fused or tacked yarns of the novel printed or dyed carpet of Figs. 3B and 3D will remain more intact, upright, tighter, have better resolution, and the like after wear or use. Consequently, the carpet of the present invention not only has better color, image, pattern, or design at printing or dyeing, but also looks better after wear or use as compared to conventional carpet.

The exemplary process for preparing the fibers, threads or yarns of the present invention will be described in more detail with reference to Figs. 4-6. In Figs. 4-6 the primary fiber or fibers, such as standard or high melt nylon 6, nylon 6,6, and/or wool, is typically provided in bales, at 100, as conventional in the art. The fibers are then passed through an opener, at 101, as known in the art. The fiber is optionally blended, at 102, with additives and adjuvants as known in the art. In one embodiment of the present invention, one or more low melt fibers 103 is incorporated with the primary fiber during the blending step, indicated at 102 in Fig. 4. After blending, the fibers or filaments are passed to a carding process, at 104. In the carding process, the non-oriented, interwoven intermingled fibers enter a pilced-roller assembly wherein, due to the difference in the longitudinal speed of the rollers the fibers are stepwise oriented and unintermingled longitudinally. This process makes the fibers relatively parallel and orders the fibers longitudinally. After carding, the fibers enter a drafting process, at 105, wherein the fibers are stretched or drawn. The drafting is typically done in three steps commonly referred to in the art as breaker drafting, intermediate drafting and finisher drafting. The stretched fiber then enters a ring spinning operation, at 106, as well known in the art.

After spinning, the fibers are doubled or wound, at 107, as known in the art. In one embodiment of the present invention, one or more low melt or low melting point fibers (LM) 108, is incorporated with the primary fiber constituents in elongate fiber form such as an elongate multifilament in the doubling operation as indicated at 107 of Fig. 5.

Strands of doubled fiber are combined in a ring twisting operation, at 109. A representative ring twisting operation is available commercially from Saco Lowell as the ROVAMATIC. In one embodiment, one or more low melt fibers (LM) 110, is incorporated with the primary fiber in elongate fiber form such as an elongate multifilament during the ring twisting operation indicated at 109 of Fig. 6.

The resultant fiber is heated, at 111, to a temperature sufficiently high to melt the low melt fiber but not high enough to melt the wool, high or standard melt fiber constituents. A melt temperature of about 60°C to about 160°C is preferred. In a particularly preferred embodiment, the fibers are heated to a temperature of less than about 120°C. The low melt fiber is preferably a polyamide although polyester and other thermoplastic materials may likewise be used. The preferred low melt polyamide is low melting point nylon 6 or nylon 6,6. One particularly preferred low melt insert fiber is 70 Denier multi-filament low melt nylon sold by Solutia having about 17 fibers per cross-section and about 4.1 denier per filament (dpf) having a round shape with a melt point of about 115°C.

The preferred standard or high melt fiber component within the yarn (i.e. the fiber that does not undergo melting) is preferably standard nylon, high melt nylon, wool or a blend of standard and/or high melt nylon and/or wool. The carpet yarn of the present invention preferably comprises spun fiber selected from a group consisting of nylon, wool, polyester, polypropylene, and blends thereof. The yarn count range is preferably about 0.5 to about 8.0 per 1 end. Most preferably the yarn number or count is about 3. The yarn preferably has a twist per inch (TPI) of about 1 to about 10.

According to one potentially desirable practice, the yarn is a two ply yarn which incorporates a low melt nylon filament intermingled with the plies. The individual plies are preferably 100% standard or high melting point nylon. Thus, according to this practice the yarns are formed substantially entirely of polyamide. By way of example, according to one contemplated practice, each ply is characterized by a single yarn number or count of about 3.10 with 5.0 twists per inch (25,4 mm) in the S direction. The plied yarn preferably is a two ply construction (two plies plus insert) having a yarn number of about 2.9 with 4.5 twists per inch (25,4 mm) in the Z direction. It is preferred that the denier per filament (dpf) range be about 0,888 to about 3.110 tex per filament (about 8 to about 28 dpf) with about 19 dpf (2.111 tex per filament) being most preferred. The yearns may be 1 to 4 ply.

For high wool content the yarn is preferably a multi-ply yarn formed of two or more singles wound with an elongate insert of low melting point polyamide or other meltable material. In one potentially desirable construction using a primary fiber blend of 25% wool and 75% nylon the single plies are characterized by a yarn number or count of about 2.20 with an "S" twist at about 4.5 twists per inch (25,4 mm) The final yarn (singles plus insert) is characterized by a yarn number of about 1.90 with a "Z" twist at about 5.75 twists per inch (25,4 mm). The wool is preferably about 25- 40 microns. It is contemplated that 1-4 plies may be used.

The low melting point material preferably makes up less than 10% and more preferably less than 5% of the final yam. According to a potentially preferred practice the low melting point material makes up about 1 percent of the final yam.

With reference to Figs. 4-6, following heat set, the yarn is staged and shipped to customers, indicated at 112, or directly tufted in a carpet backing to form tufted carpet or carpet products, such as tufted face, carpet, broadloom, runners, area rugs, carpet tile, or the like. Carpet tiles are described in U.S. Patent Nos. 4,522,857, 6,203,881, and 6,468,623. The yarn of the present invention may be used in tufted or bonded carpet. The carpet may be cut pile, loop pile, or cut and loop pile. It is preferred that it be used in a tufted cut pile carpet that is to be printed or dyed, especially jet dyed by a direct jet or indirect jet dye machine.

In one contemplated practice using a plied nylon yarn with a low melting point constituent as described above, the yarn is tufted through a woven polypropylene primary backing at a level of about 1,45 Kg/m² (43.07 ounces per square yard) and finished with a tip shear to about (1.36 Kg/m²) (40.33 ounces per square yard.) According to another contemplated practice using a plied nylon yarn with a low melting point constituent as described above, the yarn is tufted through a woven polypropylene primary backing at a level of about 1,10 Kg/m² (32.68 ounces per square yard) and finished with a tip shear to about 1,02 Kg/m² (30.33 ounces per square yard).

In one contemplated practice utilizing high wool content yarn with a primary fiber blend of 25% wool and 75% nylon and low melt insert as described above, the carpet is a tufted carpet in which the yarn is tufted through a nonwoven primary backing as will be well known to those of skill in the art. The yarn is tufted in a greige state at about 1,18 to 1,53 Kg/m² (35 to 45 ounces per square yard) and finished. Following tufting, the yarn is preferably tip sheared to remove about 0,35 mm (1/64 inch) of material and provide a uniform surface for subsequent dying and/or printing. By way of example only, in one potentially desirable product, the 25% wool, 75% nylon yarn with low melt insert as described above is tufted through a nonwoven polypropylene primary backing at about 1,35 Kg/m² (39.98 ounces per square yard) and finished to about 1.37 Kg/m² (40.42 ounces per square yard) (the backing shrinks slightly). In another potentially desirable product, the 25% wool, 75% nylon yarn with low melt insert as described above is tufted through a woven polypropylene primary backing at about 1,30 Kg/m² (38.55 ounces per square yard) and finished to about 1,22 Kg/m² (35,88 ounces per square yard).

As the manufacture of yarn and of carpet from yarn is well known in the art and has been widely practiced for decades, further elaboration and further description herein is not necessary.

Embodiments of the present invention is further directed to a process for forming a carpet comprising pixelated printing or dyeing of color, pattern, design, images, text, and/or the like thereon.

With reference to U.S. Patent No. 6120,560 and to Fig. 7 of the drawings, one schematic depiction of process steps, sequence or equipment used in one exemplary embodiment of printing or dyeing of the yarn or carpet of this invention is described and shown. A textile substrate to be patterned, 5 of Figs. 8 and 9, is first subjected to a pre-steamer, depicted at 10, which serves to bulk the yarn in the substrate in preparation for the solid shade dyeing at stage 12. The solid shade dyeing stage depicted at 12 may be carried out using various commercially available devices, so long as the devices are capable of uniformly applying and fixing a dye to a textile substrate in a single step. One way this can be achieved is by heating the dye, and applying uniformly the hot dye to the substrate in a way that allows the hot dye to fix on the substrate with no additional input of energy, as from a subsequent steaming step. For example, the dye may be applied by a series of individual nozzles or applicators that are effectively placed in close proximity to, or in contact with, the surface of the substrate. The nozzles or applicators, in turn, may be surrounded by an enclosure that allows the substrate to pass by or contact the nozzles or applicators. At the same time, the enclosure serves to prevent the dissipation of the thermal energy carried by the heated dye. The result is the dye is sufficiently hot as it contacts the substrate that it fixes almost instantaneously (actually, within a few seconds) after contacting the substrate, with no additional input of energy.

One such arrangement, which is readily available commercially, is schematically depicted in Fig. 8. Here, the substrate web 5 passes between solid shade dyer 12 and a pneumatically actuated pressure pad or bellow 32. This arrangement allows the substrate to contact the dye applicator orifice portion of dyer 12 that is positioned directly opposite bellow 32, and allows the applied heated dye to fix upon contact with the substrate.

An alternative solid shade dyeing arrangement, also using heated dye, is described in detail in U.S. Pat. No. 4,790,043 to Chappell. It is believed other means or techniques, such as using heated substrates to achieve or enhance dye fixation, would also be satisfactory under appropriate circumstances.

It has been found most effective for subsequent patterning if the color chosen during the solid shade dyeing step is relatively light and relatively neutral. Accordingly, light shades of gray or beige, particularly the latter, are preferred, although other colors and shades may be preferable, depending upon the palette of colors to be used in the patterning step and the overall patterning effect desired.

Although Figs. 7 and 8 show a solid shade dyeing step, it is to be understood that this step may be eliminated or skiped or that the yarn may be yarn dyed or solution dyed, Beck dyed, or the like. Also, a white or off white yarn (such as natural nylon or bleached wool) may go straight to the wet out application 16 or patterning device 20 and skip any solid shade dyeing or vacuuming.

Following the uniform application and fixing of dye on the substrate in the solid shade dyeing step (if any), the substrate is next passed over a vacuum slot or other means 14 to remove excess moisture, such as water and condensation resulting from the dyeing operation. Following this step, the substrate is prepared for the pattern dyeing step 20 by the application of surfactants and other chemicals 16 useful in achieving deep color penetration and distinct patterns when the patterns are applied to the substrate using highly localized, discrete streams or drops of ambient temperature liquid dye. The exact mix of chemicals at 16 will depend upon a number of factors, including the nature of the substrate, the nature and operating parameters of the patterning device used, the nature and viscosity of the dye, and other factors. The manner in which these chemicals are applied, as depicted at 16, is not critical, so long as the degree of wet pickup is satisfactory and the previously dyed surface is not adversely affected. Depending upon the results of this step, an additional, optional vacuuming stage 18 or the like may be used to remove excess moisture from the substrate prior to patterning.

Following steps 16 and/or 18, the substrate is introduced to a dye jet patterning device 20, such as depicted in Fig. 9. Substrate 5 is passed over roll 52 and onto a conveyer system that allows the substrate to pass before a series of dye applicator arrays 54. Each array is fed from a separate dye supply system, and preferably applies a different color dye. Accordingly, the eight arrays shown would provide for the use of an eight process color palette. It should be remembered, however, that a great many more than eight colors can be generated on the substrate, due to various color mixing and blending techniques. The details of the patterning device are not believed to be critical. Usually, both the substrate, as it passes through patterning device 20 and the dye applied to the substrate in patterning device 20 are essentially at ambient temperature. No effort is made to introduce thermal or other forms of energy into the dyeing process in an effort to fix, either fully or partially, any of the patterning dye until the patterning of the substrate is complete and the substrate leaves patterning device 20.

The patterning device 20 may be a broadloom patterning device as shown in Figure 9 or a carpet tile patterning device as shown in U.S. Patent No. 3,894,413. U.S. Patent No. 3,894,413 shows a jet dyeing apparatus including a supply table, jet applicator, steam chamber, water washer, hot air dryer, and collection table. Hence, carpet may be dyed in broadloom form, tile form, area rug form, runner form, or the like. Further, carpet may preferably be dyed in broadloom form and then cut into tiles, rugs, runners, area rugs, and/or the like.

Following this patterning operation, the substrate is sent, in turn, to a steamer 22, in which the dyes applied during the patterning step are fixed, then to a washer 24, where excess dyeing chemicals such as those applied at 16 may be removed, and finally to a dryer 26, where the substrate may be dried (see Fig. 7). All of these devices 22, 24, and 26 may be of any appropriate design.

It has been found that postponing the fixing of the patterning dye until the patterning is complete provides an opportunity to create an extremely rich and broad variety of color effects due to the ability to mix and blend different dyes after they have been deposited on the substrate. For example, an area on the substrate carrying unfixed dye from one of the applicator arrays can be the target of a different color dye from another of the applicator arrays, thereby providing for the in situ blending of the two different unfixed dyes. Similarly, the target for the different color dye can be selected near the edge of a previously dyed area, thereby providing for in situ dye diffusion primarily along a boundary between the two unfixed dye areas.

Because the initial solid shade is of a light, neutral color, it lends itself quite well to providing a fixed, aesthetically pleasing background against which the effects of the patterning dyes, singly and in blended combinations, can be displayed, and also appears to contribute visually and aesthetically, if not physically, to the in situ blending of the various patterning dyes on the substrate.

A particular advantage is provided in a process for manufacturing carpet wherein a yarn comprising one or more low melt fibers in combination with wool and/or one or more standard or high melt fiber constituents is dyed imagewise in a pixelated printing process. In particular, the consistency of the yarn head, as described in reference to Figs. 3B and 3D, greatly decreases the diffusion, or spread, of fibers within the yarn. As a result, individual yarn heads can be dyed independently of the adjacent yarn heads. Furthermore, the yarn heads are sufficiently discrete to allow each yarn head to receive multiple pixels of dye. The effective image resolution of the patterned image is much higher than that obtained with prior art yarns. The yarn heads of prior art yarns tend to intermingle. As a result of intermingling a single pixel of dye will be received by an individual dye head as well as those fibers from neighbouring yarn heads. As the fibers of the yarn head move the pattern becomes diffuse thereby obscuring any fine print. As a result, the carpet manufacturer has been limited to patterns which are already diffuse and which are not rendered aesthetically unpleasing when further diffused.

The carpet manufacturer has heretofore been limited to two relatively unacceptable methods for creating patterned carpet. Either the yarn is pre-colored and tufted in a pattern or the yarn is printed or dyed, such as dyed in a pixelated fashion by a Millitron^{™} jet dye machine after tufting. If pre-colored yarn is used the cost of manufacturing increases due to the demand that sufficient inventory of each colored yarn be maintained. Also, image resolution is still less than a single yarn head due to fibers intermingling between yarn heads. If the yarn is dyed after tufting, the resolution is limited due to fibers intermingling. Fibers from adjacent yarn heads are colored or they intermingle after coloring to diffuse the image. Both of these prior situations may be improved by use of the low melt content yarns of the present invention.

A dyed or patterned image is susceptible to wear as is well known in the art. With an image that is designed to be aesthetically pleasing when diffused this is of minimal concern. With a higher resolution pattern, wear is a critical concern. If the high resolution image is diffused by wear, the resolution is lost and therefore the advantages are mitigated. Therefore, one would ordinarily be expected to avoid high resolution images, or images with small pixels, due to the adverse effects of wear. It is a surprising result that a carpet manufactured according to the present invention demonstrates wear resistance, in terms of image retainability, which is superior to prior products as indicated in the following examples.

### EXAMPLE 1

A control carpet (C1) was prepared comprising 100% nylon fibers. The carpet comprised a yarn count of about 3.1, about 4.5 to 5.0 twist per inch (25,4 mm) and about 19 dpf (2.111 tex per filament).

An inventive carpet (I1) was prepared in a manner consistent with control (C1) with the exception of incorporation of a low melt fiber insert. The low melt fiber was inserted during the doubling process. A motion detector, wired to a PLC at the winding frame was incorporated to stop the spindle from doubling yarn whenever lack of movement from the low melt fiber was detected.

The control carpet (C1) and the inventive carpet (I1) were tested visually and with a Hexapod Drum Tester (ASTM D-5252) or Hexapod Tumbler (ISO/TR 10361) for the number of cycles indicated in Table 1. Each test specimen was removed every 2000 cycles for restoration by vacuuming. An electrolux upright vacuum cleaner (Discovery II) was used to make four (4) forward and backward passes along the length of the specimen. The samples were assessed using daylight equivalent vertical lighting (1500 lux). Samples were viewed at an angle of 45 degrees from a 1.5 meter distance, judging from all directions. Ratings were based on CRI TM-101 Photographic Scales with a rating index as follows: 5 = negligible or no change; 4 = slight change, 3 = moderate change, 2 = considerable change, 1=severe change. The samples were also measured for pile height before and after testing to obtain a pile height retention value.

**TABLE 1:**

| Cycles | Overall Appearance | | Color Change | | Pile Height Retention | |
|---|---|---|---|---|---|---|
| | C1 | I1 | C1 | I1 | C1 | I1 |
| 4000 | 4 | 4 | 3 | 3 | 82.9% | 80.2% |
| 12000 | 2.5 | 3 | 2 | 2 | 64.7% | 76.1% |

The specimens were visually inspected after 12,000 cycles. The inventive sample (I1) had a sharper image as visualized in a Hapsburg Pattern. The edges of lines were clearly evident in the inventive sample while the line edges were diffuse in the control sample. The yarn head tufts were clearly visible in the inventive sample while those of the control sample were not as readily visible. Color saturation and contrast were retained in the inventive sample. The color saturation and contrast of the control sample (C1) was inferior to the inventive sample (I1) both before and after testing. A visual comparison of the tested samples with untested samples revealed that the color saturation and contrast was depleted in the tested control relative to the untested (no wear) control. The color saturation and contrast remained with minimal depletion in the tested inventive sample relative to the untested (no wear) inventive sample.

### EXAMPLE 2

A control sample (C2) and inventive sample (I2) were prepared and tested as described in Example 1. The results are provided in Table 2.

**TABLE 2:**

| Cycles | Overall Appearance | | Color Change | | Pile Height Retention | |
|---|---|---|---|---|---|---|
| | C2 | I2 | C2 | I2 | C2 | I2 |
| 4000 | 4 | 4.5 | 5 | 4-5 | 91.4% | 94.3% |
| 12000 | 3 | 3.5 | 4 | 4 | 81.7% | 86.2% |

A visual evaluation, and comparison of the tested samples with untested samples, yielded results substantially similar to those recorded relative to Example 1.

In accordance with embodiments of the present invention, the addition of a "low melt" polyester or nylon (such as manufactured by Solutia) during the yarn manufacturing process (wether all one type of fiber or a blend of multi-types such as wool, nylon, a combination of these or others) results in a yarn after the heat set process that has enhanced end point definition and optical color evenness when put into a carpet base and dyed by a jet dye machine. Both staple and filament low-melts will work but the filament low-melt is preferred.

Even after extended wear tests, the carpet of the present invention shows less evidence of "sueding" - a phenomenon in typical carpet where over time the yarn bundles begin to weaken and bend, resulting in wear on the non-tip surface of the yarn resulting in worn/pulled/broken fibers. These broken fibers give a muted appearance to the carpet which changes to another shade when a hand or vacuum is run over the carpet (hence the term "sueding"). The present invention reduces this problem.

Additionally, yarn described above enhances any jet dyeing operation due to the nature of the yarn being more erect in the carpet at the dyeing process, hence the dye which is streamed to exact points on the carpet face is more apt to be applied where, and in the quantities, intended.

Other objects of the embodiments described are to enhance the dyeability of carpet, the appearance of the carpet over time, both the color and the patterning detail, and the life of the yarn bundle itself.

In at least one embodiment, the present invention addresses the problem of "sueding" in tufted carpet and increases the effective life of the carpet, especially woven carpet It also improves the dyeing of the carpet where pattern is applied by jet dyeing and the effective life of the color and pattern detail.

In at least one embodiment, the present invention provides one or more of the following advantages:

1) Extends the effective life of carpet, an advantage for the consumer and an environmental enhancement (less landfill, less recycling).

2) By being added at the beginning of the product cycle, eliminates the need for elaborate rollers, steaming and the like at pre-dyeing to stand the fiber bundles upright for dyeing.

3) Enables greater detail in dyeing patterns when combined with proprietary dyeing processes such as the Millitron^{™} jet dye machine.

4) Addresses the "sueding" problem eliminating the need for post installation shearing of carpet to remove broken or loose fibers to return the original appearance to the carpet.

5) Reduces fiber shedding.

In accordance with at least one embodiment, the present invention allows for the twist lock of multiple yarn plies together, reduces sueding of spun carpets, and allows an insert fiber to be added to yarn on existing equipment and processes.

In accordance with one example of the present invention, a nylon yarn is replaced with a nylon yarn having a low melt insert. In a more particular example, a two ply nylon yarn is replaced with a two ply nylon yarn including a low melt yarn insert added during the doubling or winding step to form a low melt containing yarn having the low melt dispersed throughout the yarn as contrasted to adding the low melt in spinning or twisting. It is preferred to use a low melt nylon, such as a nylon 6 or nylon 6,6, so that it will dye similarly to the nylon or wool of the nylon yam, wool yam, or nylon/wool blend yam.

In accordance with one example, it is preferred that the low melt fibers, filaments, threads, or yarns, represent less than about 20% by weight of the total yam, more preferably less than 10%, and most preferably less than 5%.

In a visual inspection of prior patterned carpet and patterned carpet having the low melt content of the present invention, the low melt content carpet has an over all better appearance, better color, brighter color, a little harder hand, tighter yarn heads, defined yarn heads, finer detail, and the like. After wear testing, the low melt content carpet still has better color, better resolution, tighter yarn heads, less visible wear, and the like than a prior patterned carpet subjected to wear.

In accordance with another example, a wool yarn is replaced with a wool yarn having a low melt insert.

In accordance with still yet another example, a wool/nylon blend yarn is replaced with a wool/nylon blend yarn having a low melt insert.

The invention has been described with particular emphasis on the preferred embodiments. It will be realized from the teachings herein that other embodiments, alterations, and configurations could be employed without departing from the scope of the invention which is more specifically set forth in the claims which are appended hereto.

## Claims

1. A process of forming a jet dyed carpet comprising:
a) forming at least one higher melting thread comprising at least one higher melting point fiber constituent, wherein the higher melting fiber is provided in bales;
b) passing said higher melting thread through a doubling or winding process (107) wherein a lower melting point thread is added (108);
c) spinning or twisting the higher melting thread and the lower melting point thread to form a combined thread;
d) heating (111) said combined thread above a temperature sufficient to melt said lower melting point thread;
e) after heating, tufting (206) said combined thread in a carpet backing to form a tufted carpet; and
f) printing (20) an image on said tufted carpet by a jet dye machine.

2. A jet dyed, tufted carpet comprising:
a combined thread having at least one higher melting thread comprising at least one higher melting point fiber constituent, the higher melting fiber having been provided in bales, and a lower melting point thread incorporated into the combined thread during doubling or winding, the hither melting thread and the lower melting point thread having been spun or twisted to form the combined thread,
the combined thread having been heated above a temperature sufficient to melt said lower melting point thread;
a carpet backing with the combined thread tufted therein to form the tufted carpet; and
an image printed on the tufted carpet by a jet dye machine.

3. The jet dyed carpet of claim 2 wherein said combined thread has been heated to a temperature of about 60°C to about 160°C, and preferably said temperature is no more than about 120°.

4. The jet dyed carpet of any of claims 2 or 3 wherein said lower melting point thread comprises polyamide, and said polyamide is preferably selected from a group consisting of nylon 6,6 and nylon 6.

5. The jet dyed carpet of any of claims 2 to 4 wherein said higher melting point fiber constituent is selected from the group consisting of nylon, wool, polyester, polypropylene, and blends thereof.

6. The jet dyed carpet of any of claims 2 to 5 wherein said printing has been carried out by a jet dye machine in pixelate fashion.

7. The jet dyed carpet of any of claims 2 to 4 wherein said higher melting point fiber constituent is at least one of nylon and wool.

8. The jet dyed carpet of any of claims 2 to 4 wherein said higher melting point fiber constituent is a nylon wool blend.

9. The jet dyed carpet of any of claims 2 to 8 wherein said combined thread has a yarn count of about 0.5 to about 8.0, preferably of about 1.0 to about 5.0, more preferably of about 2, or about 3.

10. The jet dyed carpet of claim 7, comprising about 0.888 to about 3.110 tex per filament (8 to about 28 denier per filament) for nylon.

11. The jet dyed carpet of claim 7 wherein said wool is about 25 to about 40 microns, preferably about 38 microns.

12. The jet dyed carpet of any of claims 2 to 11 wherein said combined thread has about 1 to about 10 twist per 2.54 cm (inch), preferably about 5 twist per 2.54 cm (inch).

13. The jet dyed carpet of claim 12 wherein said combined thread has about 5 twist per 2.54 cm (inch) and is a 1 to 4 ply.

14. The jet dyed carpet of claim 12 wherein said combined thread is plied nylon with about 4.5 twist per 2.54 cm (inch).

15. The jet dyed carpet of any of claims 2 to 8 wherein said combined thread has about 0.667-2.778 tex (about 6-25 denier) per filament, preferably about 2.111 tex (about 19 denier) per filament.

16. The jet dyed carpet of claim 15 wherein said combined thread has 1 to 4 ply not including said lower melting point thread, preferably 2 ply not including said lower melting point thread.

## Patentansprüche

1. Verfahren zum Ausbilden eines strahlgefärbten Teppichs umfassend:
(a) Bilden wenigstens eines höher schmelzenden Fadens umfassend wenigstens einen Faserbestandteil mit höherem Schmelzpunkt, wobei die höher schmelzende Faser in Ballen bereitgestellt wird;
(b) Führen des höher schmelzenden Fadens in einen Doppel- oder Wicklungsvorgang (107), bei dem ein Faden mit niedrigerem Schmelzpunkt zugesetzt wird (108);
(c) Spinnen oder Verdrillen des höher schmelzenden Fadens und des Fadens mit niedrigerem Schmelzpunkt, um einen kombinierten Faden zu bilden;
(d) Erwärmen (111) des kombinierten Fadens über eine Temperatur ausreichend, um den Faden mit niedrigerem Schmelzpunkt zu schmelzen;
(e) nach dem Erwärmen Tuften (206) des kombinierten Fadens in eine Teppichunterschicht, um einen getufteten Teppich zu bilden; und
(f) Drucken (20) eine Bilds auf den getufteten Teppich durch eine Strahlfärbemaschine.

2. Ein strahlgefärbter getufteter Teppich umfassend:
einen kombinierten Faden mit wenigstens einem höher schmelzenden Faden umfassend wenigstens einen Faserbestandteil mit höherem Schmelzpunkt, wobei die Faser mit höherem Schmelzpunkt in Ballen bereitgestellt wurde und einem Faden mit niedrigerem Schmelzpunkt, der während dem Verdoppeln oder Wickeln in den kombinierten Faden integriert wurde, wobei der höher schmelzende Faden und der Faden mit niedrigerem Schmelzpunkt gesponnen oder verdrillt wurden, um den kombinierten Faden zu bilden,
der kombinierte Faden über eine Temperatur erwärmt wurde, die ausreichend war, um den Faden mit niedrigem Schmelzpunkt zu schmelzen;
einer Teppichunterschicht mit darin getufteten kombinierten Faden, um den getufteten Teppich zu bilden; und
einem Bild, das auf den getufteten Teppich durch eine Strahlfärbemaschine aufgedruckt wurde.

3. Strahlgefärbter Teppich nach Anspruch 2, bei dem der kombinierte Faden auf eine Temperatur von ungefähr 60°C bis 160°C erwärmt wurde und vorzugsweise die Temperatur nicht mehr als 120°C betrug.

4. Strahlgefärbter Teppich nach der Ansprüche 2 oder 3, bei dem der Faden mit niedrigerem Schmelzpunkt Polyamid umfasst und das Polyamid vorzugsweise aus der Gruppe bestehend aus Nylon 6,6 und Nylon 6 gewählt ist.

5. Strahlgefärbter Teppich nach einem der Ansprüche 2-4, bei dem der Faserbestandteil mit höherem Schmelzpunkt aus der Gruppe bestehend aus Nylon, Wolle, Polyester, Polypropylen und Mischungen davon gewählt ist.

6. Strahlgefärbter Teppich nach einem der Ansprüche 2-5, bei dem der Druck durch eine Strahlfärbemaschine in pixelförmiger Art durchgeführt wurde.

7. Strahlgefärbter Teppich nach einem der Ansprüche 2-4, bei dem der Faserbestandteil mit höherem Schmelzpunkt wenigstens Nylon oder Wolle umfasst.

8. Strahlgefärbter Teppich nach einem der Ansprüche 2-4, bei dem der Faserbestandteil mit höherem Schmelzpunkt eine Nylonwollemischung ist.

9. Strahlgefärbter Teppich nach einem der Ansprüche 2-8, bei dem der kombinierte Faden einen Titer von ungefähr 0,5 bis 8,0, vorzugsweise von ungefähr 1,0 bis ungefähr 5,0, mehr bevorzugt von ungefähr 2 bis ungefähr 3 aufweist.

10. Strahlgefärbter Teppich nach Anspruch 7, umfassend ungefähr 0,888 bis ungefähr 3,110 tex pro Filament (8 bis ungefähr 28 Denier Pro Filament) für Nylon.

11. Strahlgefärbter Teppich nach Anspruch 7, bei dem die Wolle ungefähr 25 bis ungefähr 40 µm, vorzugsweise ungefähr 38 µm hat.

12. Strahlgefärbter Teppich nach einem der Ansprüche 2-11, bei dem der kombinierte Faden ungefähr 1 bis ungefähr 10 Verdrillungen pro 2,54 cm (inch), vorzugsweise ungefähr 5 Verdrillungen pro 2,54 cm (inch) aufweist.

13. Strahlgefärbter Teppich nach Anspruch 12, bei dem der kombinierte Faden ungefähr 5 Verdrillungen pro 2,54 cm (inch) aufweist und 1-4-lagig ist.

14. Strahlgefärbter Teppich nach Anspruch 12, bei dem der kombinierte Faden Lagennylon mit ungefähr 4,5 Verdrillungen pro 2,54 cm (inch) ist.

15. Strahlgefärbter Teppich nach einem der Ansprüche 2-8, bei dem kombinierte Faden ungefähr 0,667 bis 2,778 tex (ungefähr 6 bis 25 Denier) pro Filament, vorzugsweise ungefähr 2,111 tex (ungefähr 19 Denier) pro Filament hat.

16. Strahlgefärbter Teppich nach Anspruch 15, bei dem der kombinierte Faden 1 bis 4 Lagen aufweist, die keinen Faden mit niedrigerem Schmelzpunkt umfassen, vorzugsweise 2 Lagen, die keinen Faden mit niedrigerem Schmelzpunkt umfassen.

## Revendications

1. Procédé de fabrication d'un tapis teint au jet, comprenant les étapes consistant à:
a) former au moins un fil à plus haut point de fusion, comprenant au moins un élément constitutif formant fibre à plus haut point de fusion, dans lequel la fibre à plus haut point de fusion est fournie en balles ;
b) soumettre ledit fil à plus haut point de fusion à un processus de doublage ou d'enroulement (107), dans lequel un fil à plus bas point de fusion (108) est ajouté ;
c) filer ou torsader le fil à plus haut point de fusion et du fil à plus bas point de fusion pour constituer un fil combiné ;
d) chauffer (111) ledit fil combiné au-dessus d'une température suffisante pour faire fondre ledit fil à plus bas point de fusion ;
e) après le chauffage, mettre en touffes (206) ledit fil combiné dans un support envers pour former un tapis touffe ; et
f) imprimer (20) une image sur ledit tapis touffe par une machine de teinture au jet.

2. Tapis touffe teint au jet, comprenant :
un fil combiné ayant au moins un fil à plus haut point de fusion, comprenant au moins un élément constitutif formant fibre à plus haut point de fusion, la fibre à plus haut point de fusion ayant été fournie en balles, et un fil à plus bas point de fusion incorporé au fil combiné pendant un doublage ou un enroulement, le fil à plus haut point de fusion et le fil à plus bas point de fusion ayant été filés ou torsadés pour former le fil combiné ;
le fil combiné ayant été chauffé au-dessus d'une température suffisante pour faire fondre ledit fil à plus bas point de fusion ;
un support envers de tapis dans lequel le fil combiné est disposé en touffes pour former le tapis touffe ; et
une image imprimée sur le tapis touffe par une machine de teinture au jet.

3. Tapis touffe teint au jet selon la revendication 2, dans lequel ledit fil combiné a été chauffé à une température comprise entre environ 60 °C et environ 160 °C, ladite température étant, de préférence, non supérieure à environ 120°.

4. Tapis touffe teint au jet selon la revendication 2 ou 3, dans lequel ledit fil à plus bas point de fusion comprend un polyamide, et ledit polyamide est, de préférence, sélectionné à partir d'un groupe constitué par du Nylon 6,6 et du Nylon 6.

5. Tapis touffe teint au jet selon l'une quelconque des revendications 2 à 4, dans lequel ledit élément constitutif formant fibre à plus haut point de fusion est sélectionné à partir du groupe constitué par du Nylon, de la laine, du polyester, du polypropylène et de mélanges de ceux-ci.

6. Tapis touffe teint au jet selon l'une quelconque des revendications 2 à 5, dans lequel ladite impression a été exécutée par une machine de teinture au jet à la manière de points d'image.

7. Tapis touffe teint au jet selon l'une quelconque des revendications 2 à 4, dans lequel ledit élément constitutif formant fibre à plus haut point de fusion est au moins l'un du Nylon et de la laine.

8. Tapis touffe teint au jet selon l'une quelconque des revendications 2 à 4, dans lequel ledit élément constitutif formant fibre à plus haut point de fusion est un mélange de Nylon et de laine.

9. Tapis touffe teint au jet selon l'une quelconque des revendications 2 à 8, dans lequel ledit fil combiné présente un numéro de fil d'environ 0,5 à environ 8,0, de préférence d'environ 1,0 à environ 5,0 et, de manière nettement préférée, d'environ 2, ou d'environ 3.

10. Tapis touffe teint au jet selon la revendication 7, comprenant environ 0,888 à environ 3,110 tex par filament (8 à environ 28 deniers par filament) pour le Nylon.

11. Tapis touffe teint au jet selon la revendication 7, dans lequel ladite laine est d'environ 25 à environ 40 microns, de préférence d'environ 38 microns.

12. Tapis touffe teint au jet selon l'une quelconque des revendications 2 à 11, dans lequel ledit fil combiné présente d'environ 1 à environ 10 torsions pour 2,54 cm (par pouce), de préférence environ 5 torsions pour 2,54 cm (par pouce).

13. Tapis touffe teint au jet selon la revendication 12, dans lequel ledit fil combiné présente environ 5 torsions pour 2,54 cm (par pouce), et comporte de 1 à 4 brins.

14. Tapis touffe teint au jet selon la revendication 12, dans lequel ledit fil combiné est du Nylon retors comportant environ 4,5 torsions pour 2,54 cm (par pouce).

15. Tapis touffe teint au jet selon l'une quelconque des revendications 2 à 8, dans lequel ledit fil combiné représente environ 0,667 à 2,778 tex (environ 6 à 25 deniers) par filament et, de préférence, environ 2,111 tex (environ 19 deniers) par filament.

16. Tapis touffe teint au jet selon la revendication 15, dans lequel ledit fil combiné a de 1 à 4 brins, non inclus ledit fil à plus bas point de fusion et, de préférence, 2 brins non inclus ledit fil à plus bas point de fusion.
